

## UNITED STATES PATENT OFFICE

2,135,494

## ALLOY

Anthony G. de Golyer, New York, N. Y.

No Drawing. Application December 4, 1936,  
Serial No. 114,205

2 Claims.

(Cl. 75—126)

The present invention relates to a ferrous base alloy containing tungsten and boron, as well as certain other alloy elements.

The object of the present invention is to provide an alloy which is entirely or substantially free from carbon and which has a combination of advantageous physical properties and characteristics rendering it particularly valuable for use as metal cutting tools.

10 The type of alloy tool steel usually classified as "high speed" which has heretofore been in general use contains tungsten as the principal alloy element; the standard 18-4-1 high speed steel being substantially an alloy of iron with 18% tungsten, 4% chromium, 1% vanadium, 0.50% to 0.75% carbon and minor percentages of manganese and silicon. Various modifications have been proposed, such as steels containing both tungsten and molybdenum in varying ratios.

15 All of the previously known high speed steels containing tungsten or molybdenum as the principal alloy element depend upon the presence of an appreciable amount of carbon to develop the degree of hardness necessary for metal cutting tools. An examination of any of the previously known high speed steels discloses grains or particles of an excess constituent comprising a complex compound of carbon, tungsten and iron, or carbon, molybdenum and iron as the case may be. This constituent is commonly designated as the carbide segregate.

20 It is well known that a minimum carbon content of 0.50% is necessary for the development of the requisite hardness and cutting efficiency in high speed steel; the usual carbon content of such steel being from 0.60% to 0.70%.

25 I have discovered that by combining appreciable amounts of tungsten, boron, chromium and vanadium in a ferrous alloy entirely free from carbon that I can produce a composition which has a cutting efficiency superior to previously known high speed steels containing appreciable percentages of carbon. Furthermore, by reason of the freedom from carbon the alloy of the present invention is amenable to a method of thermal treatment which is markedly different from that required for heretofore known tool steels. By means of such thermal treatment 30 hardness and other physical properties and characteristics determining cutting efficiency can be accurately regulated over a wide range.

35 The essential components of the alloy of my present invention are tungsten, boron, chromium, vanadium and iron. Manganese and silicon are usually present in minor amounts. Likewise phosphorus and sulphur, as well as certain other elements commonly found in alloy steels, are usually present in ineffective amounts in the nature of incidental impurities.

The alloy of the present invention comprises tungsten 9% to 20%, boron 0.25% to 2.15%, chromium 1% to 5%, vanadium 0.50% to 4% and the remainder principally iron. Manganese and silicon will usually be present in amounts not exceeding approximately manganese 1% and silicon 1.20%.

40 I prefer to have the alloy entirely free from carbon as when this element is absent the composition is not only more amenable to thermal treatment but, in general, has greater cutting efficiency. However, by reason of the fact that certain of the materials used in the preparation of the alloy frequently contain varying amounts of carbon I have found that when my alloy is manufactured under ordinary commercial conditions it will frequently contain from about 0.03% to 0.06% carbon in the nature of an incidental impurity. I have found that such incidental carbon can be present in an amount as high as approximately 0.10% without materially decreasing the valuable physical characteristics possessed by the carbon free alloy.

45 The presence of 0.45% or more carbon in high speed steels containing tungsten as the principal alloy element results in the formation of the carbide constituent or segregate referred to hereinabove. A relatively large portion of such constituent occurring in cast ingots is in comparatively massive form which can be reduced in size and distributed throughout the steel only by mechanical working. It is well known that only the smallest particles of such carbide constituent can be dissolved in the matrix by means of heating. Consequently, a relatively large proportion of the primary carbide constituent persists through all of the thermal treatments to which such steels are subjected. Therefore, the regulation of particle size and distribution of a major portion of the complex tungsten carbide constituent forming the segregate is entirely dependent upon mechanical working. This does not provide a satisfactory method of control of the physical structure of the aggregate.

50 It has previously been proposed to employ boron as an essential component in high speed steels containing from 0.30% to 0.80% carbon. I have discovered that when effective amounts of boron, i. e. 0.15% and higher are introduced into such steels that the segregate comprises a com-

5

10

20

25

30

35

40

45

50

55

plex compound containing boron, carbon, tungsten and iron. I have found that such boro-carbide compounds are extremely hard and brittle and that relatively coarse particles of this constituent cannot be appreciably fragmented by mechanical working without rupturing the steel. I have also discovered that such boro-carbide constituents are only partially dissolved in the matrix by thermal treatment. It will be evident, therefore, that the presence of an appreciable percentage of such complex boro-carbides produces a steel in which the particle size and dissemination of the hard constituent cannot be closely regulated by thermal treatment.

In the alloy of the present invention the segregate of the cast structure appears to be essentially a complex compound of boron, tungsten and iron. This segregate can be more or less readily fragmented by mechanical working or it can be largely or entirely dissolved in the matrix by heating the cast aggregate.

Examples of alloys which I have found particularly useful for metal cutting tools contain tungsten 14%, boron 0.75%, chromium 3.60%, vanadium 1.50%, manganese 0.40%, silicon 0.60% and the balance substantially iron; tungsten 18%, boron 0.95%, chromium 3.90%, vanadium 1.80%, manganese 0.50%, silicon 0.55%, carbon 0.05% and the balance substantially iron.

I have found that the hardness and other physical properties and characteristics of the alloy can be accurately controlled by means of suitable thermal treatment. As an illustration one satisfactory method consists essentially of heating an aggregate of the alloy to a temperature in excess of 1000° C.; maintaining the aggregate at such temperature for a sufficient period of time to dissolve an appreciable proportion of the tungsten-boron-iron segregate in the matrix; quenching the aggregate to substantially retain the solid solution; subsequently heating the aggregate to a temperature substantially lower than that at which the solid solution was formed for a sufficient period of time to produce precipitation of tungsten-iron-boride particles from the solid so-

lution. I have found that in carrying out the primary heating for effecting solid solution it is not necessary to dissolve all of the tungsten-iron-boride constituent in the matrix. After the alloy has been quenched from the primary heating temperature it will usually have a hardness of approximately 48 to 52 Rockwell C compared to a hardness of from 62 to 70 Rockwell C which can be developed by precipitation of the tungsten-boron containing constituent during the secondary heating. It will be apparent that by regulating the temperatures and periods of heating the ratio of precipitated boron compound to matrix constituent, or to primary boron compound may be accurately controlled. The precipitated boron compound is uniformly disseminated throughout the aggregate.

I have found that the boron containing constituent of the present alloy is not only extremely hard but is relatively strong. The presence of boron imparts high impact strength to the alloy, particularly at temperatures generated in the tip of a metal cutting tool. Such boron containing compounds are also highly resistant to oxidation at such temperatures, and consequently the injurious effect of decarburization, which occurs in carbon containing tools, is entirely eliminated.

Although the greatest scope of usefulness of this alloy appears to be in cast or wrought forms as cutting tools, I have found it may be used for many other industrial applications such as forming dies, wearing parts, etc.

I claim:

1. An alloy containing tungsten 9% to 20%, boron 0.25% to 2.15%, chromium 1% to 5%, vanadium 0.50% to 4%, manganese not exceeding approximately 1%, silicon not exceeding approximately 1.20% and the remainder iron.

2. An alloy containing tungsten 9% to 20%, boron 0.25% to 2.15%, chromium 1% to 5%, vanadium 0.50% to 4%, manganese not exceeding approximately 1%, silicon not exceeding approximately 1.20%, carbon not exceeding approximately 0.10% and the remainder iron.

ANTHONY G. DE GOLYER. 45